

T. S. FULLER.

COMPOSITE METAL.

APPLICATION FILED JAN. 29, 1913.

1,077,977.

Patented Nov. 11, 1913.



WITNESSES :

J. Earl Ryan.  
J. Ellis Green.

INVENTOR :

TRUMAN S. FULLER,

BY *Albert H. Davis*  
HIS ATTORNEY.

# UNITED STATES PATENT OFFICE.

TRUMAN S. FULLER, OF SCHENECTADY, NEW YORK, ASSIGNOR TO GENERAL ELECTRIC COMPANY, A CORPORATION OF NEW YORK.

## COMPOSITE METAL.

1,077,977.

Specification of Letters Patent.

Patented Nov. 11, 1913.

Application filed January 29, 1913. Serial No. 744,807.

To all whom it may concern:

Be it known that I, TRUMAN S. FULLER, a citizen of the United States, residing at Schenectady, in the county of Schenectady 5 and State of New York, have invented certain new and useful Improvements in Composite Metals, of which the following is a specification.

My invention relates to duplex or composite metals and more particularly to metals of this character in which a copper-nickel alloy having nickel predominating is united to a ferrous metal in which iron predominates in such a way that the composite body 15 of metal may be rolled, drawn and otherwise treated as a single metal.

Nickel-copper alloys in which nickel predominates possess properties which are very useful in the arts. This is particularly true 20 of a metal of this class commercially known as "Monel" metal which is a natural alloy containing nickel, copper and a small percentage of other metals such as iron and manganese, the ratio of nickel and copper 25 being about 2 to 1. This metal is non-oxidizable, even at a very high temperature, is not affected by atmospheric conditions, and resists the corrosive action of acids, salt water, etc. It is very strong, hard, ductile, 30 and is susceptible of a very high polish. The relatively high cost of this metal and the fact that it is not as easily workable as some more commonly used metals however tends to limit its use in the arts.

One of the objects of my invention is to 35 form a composite metal by uniting a metal of the general character of Monel metal to a less expensive metal such as iron or steel, so that the composite metal will have most 40 of the essential properties of the Monel metal but will be less expensive and more easily workable.

I have found that a nickel-copper alloy in 45 which nickel predominates may be united under certain conditions to another metal in which iron predominates by an intermediate cupreous film or layer. The composite metal thus formed may be rolled, drawn or otherwise worked as a single metal since 50 the metals are so thoroughly united that they act as one metal. I have found, for instance, that a plate of the aforesaid alloy may be united to a plate of iron or steel by inserting a sheet of copper between the 55 plates and raising the temperature to the

melting point of copper in a non-oxidizing atmosphere, no compression of the plates and no flux of any kind being required.

In the drawing is illustrated an arrangement of plates and sheets of metals preparatory to placing the same in a furnace for the purpose of carrying out my invention.

The object is to produce a composite billet consisting of a layer of iron or steel coated on both sides with a film or layer of the nickel-copper alloy.

10 is a plate of iron or steel. I have found that a steel comprising about 13/100% carbon and 36/100% manganese is very suitable for this purpose.

11 and 12 are plates of nickel-copper alloy in which nickel predominates. 13 and 14 are sheets of copper. The superposed bodies of metal are placed in a furnace and raised to substantially the melting point of 75 the copper or somewhat above, but below the melting points of the other metals. This should be done in a non-oxidizing or inert atmosphere. A hydrogen atmosphere is particularly desirable as it readily reduces 80 any oxids on the surface of the metals. However the process may be carried out in an electric vacuum furnace utilizing carbon electrodes.

After the above-stated operation has 85 progressed sufficiently to thoroughly melt the copper the composite billet may be removed from the furnace. It will be found that the metals are very intimately joined and even a microscopic examination will 90 disclose practically no flaws. The composite billet may be readily worked as by rolling without effecting a separation of the component metal layers, and the rolling may be conducted at a high temperature or 95 at a low temperature. On account of the fact that the nickel-copper alloy is not heated to an excessive temperature during the melting operation it suffers no deterioration from such operation. This is im- 100 portant because it is known that such alloys are injured by high temperatures. A billet of this kind may be rolled down to very thin sheets and it will be found that the relative thicknesses of the alloy and iron or 105 steel are substantially the same in the final sheet as they are in the original billet.

A composite sheet metal embodying my invention may be used for a variety of purposes on account of the fact that it is easy 110

to work, is comparatively inexpensive and possesses the advantages of Monel metal to a high degree. It can be fashioned into articles of various shapes as it lends itself readily to the spinning or rolling processes. The coating of nickel-copper alloy protects the iron or steel from corrosion. For this reason the composite metal is suitable for use in making cooking utensils, crucibles, water tanks, and in fact, any article which is subjected in use to oxidizing or corroding agents.

A very important use for this metal is for roofing purposes. Another is for making or lining ovens or other portions of heating devices which are subjected to comparatively high temperatures. It is especially adapted for making ovens for electrically heated ranges for the reason that in such ovens the heat is localized and causes their very rapid deterioration if constructed of iron or steel or other commonly used metals.

Another composite metal body may be formed by the process herein described the said composite metal body consisting of a metal sheet containing a layer of Monel metal and a layer of high resistance alloy. An example of such alloy which has been found to unite very readily to the Monel metal by my process contains 77% iron,

17% nickel, 4% chromium, and 2% manganese.

Various changes and modifications of my invention will readily suggest themselves to those skilled in the art and are to be considered as coming within the scope thereof as set forth in the following claims.

What I claim as new and desire to secure by Letters Patent of the United States, is:

1. A composite metal body comprising a layer consisting mainly of iron and a layer of an alloy of nickel and copper in which nickel predominates, the said layers being intimately united by a cupreous film or layer.

2. A composite metal body comprising a layer of steel, a layer of an alloy of nickel and copper in which nickel predominates and an intermediate cupreous layer or film, the said layers being intimately joined.

3. A composite metal body comprising a plate of ferrous metal having a sheet of nickel-copper alloy united to each side thereof by a layer of copper.

In witness whereof, I have hereunto set my hand this 27th day of January, 1913.

TRUMAN S. FULLER.

Witnesses:

BENJAMIN B. HULL,  
HELEN ORFORD.